

Aug. 21, 1928.

J. C. TAYLOR, JR.

1,681,906

BUSHED MANGANESE STEEL SHEAVE AND THE LIKE

Filed Sept. 21, 1927

*Fig. 1.*



*Fig. 2.*



JOHN C. TAYLOR, JR.,

By *Jack Richmond*

Attorney

## UNITED STATES PATENT OFFICE.

JOHN C. TAYLOR, JR., OF HIGH BRIDGE, NEW JERSEY, ASSIGNOR TO TAYLOR-WHAR-  
TON IRON AND STEEL COMPANY, OF HIGH BRIDGE, NEW JERSEY, A CORPORATION  
OF NEW JERSEY.

## BUSHED MANGANESE-STEEL SHEAVE AND THE LIKE.

Application filed September 21, 1927. Serial No. 220,958.

The invention relates more particularly to the production of manganese steel gears, sprockets, sheaves, pulleys and the like. Manganese steel is substantially non-machinable and heretofore it has been the practice to provide elements of the nature indicated with separately formed or with integrally cast machinable bushings. Both expedients are objectionable, especially that which provides for anchoring the bushing in the act of casting. Under such condition, the manganese steel must be excessively heavy in the hub and hence in the balance of the casting in order to prevent cracking when shrinking around the soft steel or other machinable bushing.

It is the object of my invention to obviate the disadvantages of the old practice and more particularly to eliminate excessively heavy manganese steel sections in bushed castings of the character stated.

The nature of the invention consists in the provision of an integrally cast manganese steel gear, sheave or the like wheel element having a machinable bushing locked in the bore of the hub, in the act of casting, the bushing being divided longitudinally for the purpose and with the result of contracting as the manganese steel shrinks around it in the act of casting or in the act of heat treatment.

The preferred embodiment of the invention is illustrated in the accompanying drawing, wherein

Figure 1 is an end view of the improved bushed wheel.

Fig. 2 is a section on line 2—2 of Fig. 1.

In the drawings, numeral 5 represents a solid or integrally cast gear, sheave, or the like, having spokes terminating in a hub 6, whereof the bore is formed by a bushing 7 secured to place in the act of casting the main body. The wheel body or main casting is constructed of manganese steel or other substantially non-machinable or difficultly machinable steel. The bushing is constructed of soft steel or other machinable metal and is further characterized by a longitudinal di-

vision which provides an endwise ranging gap or space 8, to permit the bushing to contract in response to shrinkage of the wheel casting and, hence, to afford a relief to shrinkage strains. The line of division is preferably on a bias in order to obtain the maximum of contraction, if necessary, by thus providing for relative sliding movement of the overlapping ends.

The bushing is equipped with radial projections 9 which are surrounded by metal of the wheel casting and thus positively lock the bushing to place.

Having described my invention, I claim:

1. The method of eliminating excess metal and otherwise to insure uniformity of sound metal section in wheel shapes of manganese steel or other substantially non-machinable metal, which consists in moulding the shape around a machinable bushing having spaced longitudinal wall sections whereby it is free to contract to relieve strains incidental to shrinkage of the manganese steel.

2. A wheel shape of substantially non-machinable metal having a machinable center or bushing interlocked therewith in the act of casting, said bushing having a single longitudinal line of division to form an intervening gap whereby it constitutes a relief to shrinkage of the non-machinable metal.

3. A wheel shape of substantially non-machinable metal having a machinable center or bushing interlocked therewith in the act of casting, said bushing having a longitudinally ranging biased line of division whereby it constitutes a relief to shrinkage of the non-machinable metal.

4. A wheel shape of manganese steel having a one-piece machinable center incorporated in the act of casting, said center consisting of a tube having spaced longitudinal walls in overlapping and underlapping relation to permit appreciable separation or conversely abutting relation without disturbing the bridging relation of the walls.

In testimony whereof I affix my signature.

JOHN C. TAYLOR, JR.